

# UNITED STATES PATENT OFFICE.

CHARLES EDOUARD GUILLAUME, OF SÈVRES, FRANCE, ASSIGNOR TO SOCIÉTÉ DES FABRIQUES DE SPIRAUX RÉUNIES, OF LA CHAUX-DE-FONDS, SWITZERLAND.

## BALANCE-SPRING HAVING ELASTICITY INCREASING WITH RISE IN TEMPERATURE.

1,106,207.

Specification of Letters Patent.

Patented Aug. 4, 1914.

No Drawing.

Application filed February 20, 1912. Serial No. 679,303.

*To all whom it may concern:*

Be it known that I, CHARLES EDOUARD GUILLAUME, doctor of philosophy and assistant director of the International Office of Weights and Measures, a citizen of the Swiss Republic, and resident of Sèvres, Department of Seine-et-Oise, France, have invented new and useful Improvements in Balance-Springs Having Elasticity Increasing with Rise in Temperature, of which the following is a full, clear, and exact specification.

For some years escapements for watches, clocks, etc., have been used comprising a balance wheel which is not cut and a spring of elasticity increasing with the temperature so that it compensates for the variations of the inertia of the balance wheel with variations of temperature. Hitherto there have been used for this purpose practically only balance springs of nickel-steel containing 27-28 per cent. of nickel as specified in United States Letters Patent 669,763 dated March 12, 1901. This steel being very soft springs made of it have a very low elastic limit and consequently are very easily deformed, especially if they are not made with great care; moreover, the soft character of this alloy makes the construction of the escapement and the operation of regulating it very delicate. It follows that these escapements cannot be used for accurate watches intended for chronometric computations in observatories.

This invention relates to a balance spring having elasticity increasing with the rise of temperature, which possesses a high elastic limit. This result is obtained by making balance springs of an alloy of iron and nickel containing from 27-31 per cent. of nickel, 0.3 to 0.6 per cent. of silicon, 0.3 to 0.6 per cent. of carbon, at least one metal of the sixth group of the classification of Mendeléeff, as for instance, chromium, molybdenum or tungsten and at least one metal of the fifth group of the said classification, as for instance, vanadium or tantalum, the said metals being each employed in a quantity of 0.2 to 4 per cent. in such a manner that the total amount of them and of the carbon and silicon comprises between 3.5 to 10 per cent. of the whole alloy. The alloy can also contain 1 to 4 per cent. of manganese, in which case the total amount of carbon, of silicon, of manganese and of the other metals added to

the alloy of nickel and iron must always remain between 3.5 to 10 per cent. of the whole alloy. When so made the balance spring has a high elastic limit and also the property of increasing in elasticity as the temperature rises; consequently it may be used in the construction of the escapement without risk of undergoing any deformation and lends itself to the operation of regulating the escapement as easily as the steel springs of ordinary escapements do.

By way of example the composition of an alloy for balance springs according to this invention is given hereafter:

|           |      |                  |    |
|-----------|------|------------------|----|
| Nickel    | 30.5 | parts by weight. | 70 |
| Iron      | 61.6 | " "              |    |
| Manganese | 4    | " "              |    |
| Chromium  | 1.8  | " "              |    |
| Vanadium  | 1.0  | " "              |    |
| Carbon    | 0.6  | " "              | 75 |
| Silicon   | 0.5  | " "              |    |

What I claim is:

1. A balance spring, of which the elasticity increases with the rise of temperature and with a high elastic limit consisting of an alloy of iron and nickel containing between 27-31 per cent. of nickel and besides of small quantities of carbon and of silicon at least one metal of the sixth group of the classification of Mendeléeff and at least one metal of the fifth group of the said classification, each of these metals being in such a proportion between 0.2 and 4 per cent., that the total amount of these metals and of the carbon and silicon in the alloy is between 3.5 and 10 per cent. of the whole alloy.

2. A balance spring of which the elasticity increases with the rise of temperature and which has a high elastic limit made from an alloy of iron and nickel containing between 27-31 per cent. of nickel and besides of small quantities of carbon and of silicon and of 1 to 4 per cent. of manganese at least one metal of the sixth group of the classification of Mendeléeff and at least one metal of the fifth group of the said classification, each of these metals being in such a proportion between 0.2 and 4 per cent., that the total amount of these metals and of the carbon manganese and silicon in the alloy is between 3.5 and 10 per cent. of the whole alloy.

3. A balance spring, of which the elasticity increases with the rise of temperature

105  
110

and which has high elastic limit consisting of an alloy of iron and nickel containing between 27-31 per cent. of nickel and besides of small quantities of carbon and of silicon 5 chromium and a metal of the fifth group of the classification of Mendelejeff, each of these metals being in such a proportion between 0.2 and 4 per cent., that the total amount of these metals and of the carbon and silicon in the 10 alloy is between 3.5 and 10 per cent. of the whole alloy.

4. A balance spring of which the elasticity increases with the rise of temperature and which has a high elastic limit consisting of 15 an alloy of iron and nickel containing between 27-31 per cent. of nickel and besides of small quantities of carbon and of silicon and of 1 to 2 per cent. of manganese chromium and a metal of the fifth group of the 20 classification of Mendelejeff, each of these metals being in such a proportion between 0.2 and 4 per cent., that the total amount of these metals and of the carbon, manganese and silicon in the alloy is between 3.5 and 10 per 25 cent. of the whole alloy.

5. A balance spring of which the elasticity increases with the rise of temperature and which has high elastic limit consisting of an alloy of iron and nickel containing between

27-31 per cent. of nickel and besides of small 30 quantities of carbon and of silicon, chromium and vanadium, each of these metals being in such a proportion between 0.2 and 4 per cent., that the total amount of these metals and of the carbon and silicon in the 35 alloy is between 3.5 and 10 per cent. of the whole alloy.

6. A balance spring of which the elasticity increases with the rise of temperature and which has high elastic limit consisting of 40 an alloy of iron and nickel containing between 27-31 per cent. of nickel and besides of small quantities of carbon and of silicon and of 1 to 4 per cent. of manganese, chromium and vanadium, each of these metals 45 being in such a proportion between 0.2 and 4 per cent., that the total amount of these metals and of the carbon, manganese and silicon in the alloy is between 3.5 and 10 per cent. of the whole alloy.

In witness whereof I have hereunto signed my name this 7th day of February, 1912, in the presence of two subscribing witnesses.

CHARLES EDOUARD GUILLAUME.

Witnesses:

CHARLES ALBERT VUILLE,  
BARTLEY F. YOST.